

# UNITED STATES PATENT OFFICE.

WENDELL G. WILCOX, OF LAKEWOOD, OHIO, ASSIGNOR TO NATIONAL CARBON COMPANY, OF CLEVELAND, OHIO, A CORPORATION OF NEW JERSEY.

## PROJECTOR-CARBON.

1,186,253.

Specification of Letters Patent.

Patented June 6, 1916.

No Drawing.

Application filed July 2, 1913. Serial No. 777,128.

To all whom it may concern:

Be it known that I, WENDELL G. WILCOX, a citizen of the United States, residing at Lakewood, in the county of Cuyahoga and 5 State of Ohio, have invented a certain new and useful Improvement in Projector-Carbons, of which the following is a full, clear, and exact description.

This invention relates to non-flaming are 10 light electrodes particularly adapted for projection work.

The object of the invention is to constitute the electrode or its core so that the crater will not travel to any extent and its 15 temperature will not vary through any wide range.

Many salts and oxids have been used in 20 arc light electrodes to increase the candle-power of the arc itself. In the old carbon arc the greater part of the light came from the crater in the electrode. The flaming type of arc lamp, however, derives most of 25 its light from the arc itself. Hence, the salts, oxids and other materials added to the electrodes have not been used for the purpose 30 of maintaining the crater in any definite position, or for increasing its temperature. Consequently the flaming arc, though admirably suited for street and other general 35 lighting cannot be used for projection work, as the crater is constantly moving, and the arc itself undergoes so many changes that it is unsuitable for this work. Changes in the candle-power or in the position of the 40 crater in a flaming arc lamp are small enough to be of no consequence in street lighting, but the changes are very undesirable when used in projection work.

It is known that potassium or sodium silicate tends to steady the arc, but I have found 45 that the steadiness will be increased to a much greater extent if other salts are used in combination with the potassium or sodium silicate. If potassium titano-fluorid ( $K_2TiF_6$ ); potassium silico-fluorid ( $K_2SiF_6$ ), or potassium zircono fluorid ( $K_2ZrF_6$ ), be used alone or together with potassium silicate the crater of the arc is much more 50 stationary than if potassium silicate is used alone or with any other salts that I have tried out. The temperature of the crater is likewise more constant and the unpleasant flickering on a moving picture screen for instance is practically eliminated.

The electrodes may be made of carbon, 55 such as gas coke, petroleum coke, lampblack or other forms of carbon, and may have a core consisting of about 80% of carbon, 19% to 15% potassium silicate and 1% to 5% of either of the fluorin compounds above given. 60 Instead of using the fluorin salts mentioned alone in combination with the potassium or sodium silicate the three may be combined in varying amounts so that the combination will consist of from 1% to 5% of the core 65 mass.

While it is preferred to place the salts mentioned in the core of the electrode in some cases, it may be desirable to incorporate the salts and the carbon as a homogeneous mixture. However, for moving picture work this would not be the preferred form. The potassium salts have been given as the examples in the previous description, but sodium salts may also be used either as 75 the silicate or as the fluorid compounds.

For the purpose of this application the terms "alkaline" and "double fluorid" in the claims are intended to cover only those examples disclosed and their equivalents.

While I prefer to use the double fluorids and alkaline silicates within the limits given, these compounds suit the purpose when used within still wider limits. For instance I have obtained good results when as low as 85 10% of the silicates and as high as 10% of the double fluorids were used.

Having described my invention what I claim is:

1. A projector carbon containing a carbon body, 19 to 10 parts alkaline silicate and 1 to 10 parts of double fluorids.

2. A projector carbon having a carbon shell, a core therefor containing 80% carbon, 19 to 10 parts alkaline silicate, and 1 to 10 95 parts of double fluorids.

3. A projector carbon containing a carbon shell and a core consisting of 19 to 10 parts potassium silicate and 1 to 10 parts potassium-silico-fluorid.

In testimony whereof, I hereunto affix my signature.

WENDELL G. WILCOX.

Witnesses:

GLEN P. COWAN,  
CHARLES W. HILL,